

## UNITED STATES PATENT OFFICE

1,947,981

## PLATING ALUMINUM

Johannes Fischer, Berlin-Charlottenburg, Germany, assignor to Siemens & Halske Aktiengesellschaft, Siemensstadt, near Berlin, Germany, a corporation of Germany

No. Drawing. Application October 31, 1931,  
Serial No. 572,440, and in Germany November  
6, 1930

4 Claims. (Cl. 204—3)

This invention relates to plating aluminum; and it comprises a method of electrically plating articles of aluminum and aluminum alloys with other metals wherein such an article is electrolytically treated until an oxidized film develops, is thereafter made a cathode in an alkaline solution containing a depositable metal until the oxidized film is partially removed and a very thin plating of said metal is formed and is thereafter electrolytically coated with metal deposited on said very thin plating; said very thin plating being usually either copper or brass; all as more fully hereinafter set forth and as claimed.

As is well known, it is impracticable to produce good electric platings of other metals on articles made of aluminum or aluminum alloy, by known methods. This is for the reason that all such articles on exposure to the air become covered with a coherent, very thin film of oxidized nature; this instantly renewing itself on abrasion. It is therefore impracticable by buffing or other similar treatments to prepare and maintain a true metallic surface on an article at the time when it is immersed in a plating bath. In plating, this oxid coating must be disposed of in some way prior to deposition of metal; and this disposition is extremely difficult in the usual methods of plating and in the usual plating baths.

In the present invention I use an expedient which consists in first producing an oxidized coating of different nature and afterwards simultaneously partially removing it and depositing a film coating of another metal on the aluminum as the coating is partially removed. The metal of the film coating produced in this way sticks to the surface.

As is well known, aluminum when made an anode in many solutions becomes covered with a protective coating of oxidized nature having a unilateral conductivity; a phenomenon which permits the use of aluminum in rectifiers and "wet electrical condensers". This coating is different from the "air-film" always occurring on aluminum and enables the production of a metallic coating on the aluminum if the coated articles are subsequently treated by the process hereinafter described.

I have found that by providing aluminum with such an anodic coating, the coating can be partially removed when the article is made a cathode in an alkaline bath and if the bath contains a metal which can be deposited, simultaneously with the partial removal of the oxid coating I can deposit this metal in the form of an adherent film coating. The metal placed in solution in the

bath to form the film coating can be any of those usually deposited as foundations for galvanic coatings. In practice, we use a bath depositing either copper or brass; that is, for example, a bath containing double cyanides of copper and alkali, or of copper and alkali and of zinc and alkali, as the case may be. Cadmium plating baths may be used.

The film coating deposited from an alkaline bath, although very thin, adheres well to the underlying layer. The film coating can be afterwards plated in the regular way in any convenient bath with no more difficulty than an article of the same kind made of copper, or of brass, as the case may be.

In practice, the metal for the film coating is best copper or brass, although cadmium, silver or gold can be used if desired. The metal for the main coating may be any of the usual metals deposited by electroplating that is, copper, brass, gold, silver, nickel, chromium, cadmium, etc. The present process is applicable to the coating of aluminum with any metal which may be desired for decoration or protection.

Where alternating current is used for the primary oxidation the first and second step of the process may be conducted in a single bath; the article being first provided with an electrochemically produced oxid coating by connection with an alternating current. Then the alternating current is replaced by a direct current, the article being made a cathode.

In providing the oxid coating, which is the first operation in our process, either alternating or direct current may be used; the article being made an anode in the latter event.

In practical embodiments of this invention, using direct current throughout one may employ for the oxidizing treatment a bath containing an oxidizing organic or inorganic acid. A 30 to 40 per cent solution of chromic acid containing some sulfuric acid is suitable. A voltage of 20 to 60 volts may be employed. After production of the oxid coating, this is partially removed and an extremely thin coating of copper or brass simultaneously deposited thereon in an alkaline bath. The article is made a cathode and voltage may be applied as is necessary, that usually used being ordinarily over 5 volts. After formation of the primary metallic or film coating, the main coating is applied.

In a practical embodiment of the described invention, an article of aluminum is made an anode for 15 to 30 minutes in a chromic acid bath of the kind described. This converts the usual

60

65

70

75

80

85

90

95

100

105

110

air film on the aluminum into a different type of coating, also of oxidized nature. After forming the oxid coating the article is removed from the chromic acid bath, washed and made a cathode 5 at about 6 volts in an alkaline bath adapted for the deposition of brass. After two to three minutes passage of the current enough metal is deposited on the aluminum in adherent relationship therewith to serve as a basis for subsequent plating. After washing, the article may be directly plated with any desirable metal among those 10 named hereinbefore.

In another practical embodiment of our invention an aluminum article is placed in a bath containing double copper-alkali cyanids and zinc-alkali cyanids, together with a counter electrode of sheet iron and an alternating current is imposed. This current may be at 30 to 40 volts and the current density may be 800 amperes per 15 square meter. After two minutes exposure to alternating current, direct current is substituted, making the aluminum a cathode without changing the treating bath. With 5 volts and a current density of 300 amperes per square meter, in about 20 five minutes it is found that the oxid coating is partially removed and an extremely thin skin of brass is deposited on the article. The brassed article may be removed from the bath and plated with gold, copper, brass, tin, silver, nickel, chromium, cadmium, etc., in any suitable bath. 25

Plated aluminum articles produced under the present invention may be buffed, polished and otherwise finished in the usual ways. 30

What is claimed is:

1. In brass coating articles made of aluminum and aluminum alloys, the process which comprises imposing alternating current on such an article in a brassing bath containing double cyanids of copper and alkali and of zinc and alkali, continuing such current until an oxidized coating is produced, substituting a low potential direct current with the article a cathode for the alternating current and then finish plating the article in 80 the usual manner.
2. In the plating of articles of aluminum and of aluminum alloys with firmly coherent, substantial metal coatings, the process which comprises passing an electric current between such articles through a bath containing electrolytes of such 85 nature as to produce an electrolytic coating of oxidized nature, flash coating the so-treated articles electrolytically in an alkaline bath with a metal selected from a group consisting of copper, brass, cadmium, silver and gold, and finish-coating said flash-coated articles electrolytically. 90
3. The process of claim 2 wherein the said flash-coating is produced in an alkaline cyanide bath. 95
4. The process of claim 2 wherein the coating of oxidized character and the flash-coating are produced in the same bath, the coating of oxidized character being produced by alternating current. 100

JOHANNES FISCHER. 105

37

110

40

115

45

120

50

125

55

130

60

135

65

140

70

145

75

150